

Nov. 21, 1933.

E. M. WISE

1,935,897

PRECIOUS METAL ALLOY

Original Filed Jan. 28, 1929

2 Sheets-Sheet 1

*Fig. 1.*



*Fig. 2.*



INVENTOR

Edmund M. Wise

BY

Bynes, Stibbs, Parmenter, & Blenko

ATTORNEY

Nov. 21, 1933.

E. M. WISE

1,935,897

PRECIOUS METAL ALLOY

Original Filed Jan. 28, 1929

2 Sheets-Sheet 2

Fig. 3.



Fig. 4.



Fig. 5.



The effect of Cumulative Aging (30 Min. at each Temp.)  
on the Hardness of  
Palladium Alloys. All Alloys Quenched from 860°C

INVENTOR

Edmund M. Wise

BY

Byers, Stalbin, Parmelle & Blenko

ATTORNEY

## UNITED STATES PATENT OFFICE

1,935,897

## PRECIOUS METAL ALLOY

Edmund M. Wise, Jersey City, N. J., assignor to  
The International Nickel Company, Inc., a corporation of Delaware

Original application January 28, 1929, Serial No.  
335,481. Divided and this application December 30, 1929. Serial No. 417,335

7 Claims. (Cl. 75—1)

This invention relates to improved alloys of palladium, silver and copper, and to a novel method of heat-treating the same, and more particularly to alloys of the above metals having a high tarnish and corrosion resistance, a high hardness value and other characteristics which render them especially suitable for dental use, and for other advantageous uses such as heat and electrical conductors.

One of the objects of the invention is to provide an improved metal alloy which is white in color, which is resistant to corrosion, and which is both strong and ductile.

Another object is to provide a metal alloy which is particularly adapted for dental, and electrical and heat conductive purposes.

Still another object is to provide an alloy having a high resistance to tarnish, and one having a comparatively high hardness value and tensile strength.

The invention also consists in certain new and original features of treatment and combinations of elements hereinafter set forth and claimed.

Although the novel features which are believed to be characteristic of this invention will be particularly pointed out in the claims appended here-to, the invention itself, as to its objects and advantages, the mode of its operation and the manner of its organization may be better understood by referring to the following description taken in connection with the accompanying drawings forming a part thereof, in which Fig. 1 is a ternary diagram showing the range in composition of an alloy of palladium, silver and copper in accordance with the present invention;

Fig. 2 is a ternary diagram showing the composition of the alloys divided in accordance with tarnish resistance;

Fig. 3 is a ternary diagram showing the range of hardenable alloys;

Fig. 4 is a ternary diagram showing the range of alloys which are particularly suitable for dental purposes; and

Fig. 5 is a graphic diagram showing the effect of heat treatment at various temperatures on the hardness of certain alloys.

In the following description and in the claims elements will be identified by specific names for convenience, but they are intended to be as generic in their application to similar elements as the art will permit.

In accordance with the present invention alloys consisting of palladium, silver and copper have been found to have a resistance to tarnish and corrosion which is dependent upon the relative

percentages of the various metals and sometimes upon the heat treatment to which they are subjected. Alloys lying in the area ABC of the diagram of Fig. 2 have been found to be substantially completely resistant to both tarnish and corrosion. Alloys lying in the area DEBA of that diagram are largely resistant to tarnish and corrosion and may be considered within a useful range, while the remaining alloys possess this property to a less degree.

The area ABC may be approximately represented analytically by stating that the palladium represents from 35% to 98% and is not less than  $35 + (6/7 \times \% \text{ Cu})$ , the copper content being not less than 1% and the silver constituting substantially the remainder of the alloy, but being not less than 1% of the total. The area of useful alloys represented as DEC on the diagram may be defined analytically as containing from 25% to 98% palladium, the palladium content being not less than  $25 + (4/11 \times \% \text{ Cu})$ , the copper being not less than 1% with the silver constituting substantially the remainder of the alloys, but being not less than 1%.

The resistance to corrosion and tarnish represented by the curves of Fig. 2 was determined by subjecting the alloys to moist  $\text{H}_2\text{S}$  vapor. The arrangement used consisted of a desiccator containing a solution of sulphuric acid in water (43%  $\text{H}_2\text{SO}_4$  by wt.). This solution will maintain 50% relative humidity in the desiccator. A small beaker containing a solution of sodium polysulphide was also placed in the bottom of the desiccator which maintains a small concentration of  $\text{H}_2\text{S}$  in the chamber. It should also be noted that the vapor also contains a trace of  $\text{H}_2\text{SO}_4$ . The samples prepared by polishing and rubbing with dry alumina were placed on a tray in the desiccator and allowed to remain fifteen hours or longer as indicated. The specimens were then removed and half of the specimen rubbed with alumina to remove any tarnish that might be present.

The amount of tarnish was then noted and utilized in the formation of the above mentioned diagram. This particular type of a tarnish test is employed because it is the one in common use in the dental trade and is the well known means for classifying alloys as to their tarnish resistance properties.

It has been found that certain alloys may, by suitable heat treatment, have their hardness and tensile strength materially increased. It has also been found that the heat conductivity and electrical conductivity of the hardenable alloys

can be increased by a precipitation heat treatment. Referring to Fig. 3, the alloys in which substantial hardening will take place upon heat treatment are represented by a portion of the 5 area above the dotted line in that figure. It may be approximately represented analytically by stating that the palladium content varies between the limits of 25% and 62.6% with the copper percentage greater than  $5 + 1.544 \times 10^{-3}$  (Pd—35)<sup>3</sup> 10 and less than 48%, with silver constituting substantially the remainder of the alloy. The solid curves represent alloys that have been hardened to Rockwell B values of 80-110.

It will be understood that the temperatures for 15 heat treatment may be varied within considerable limits. Desired results have been obtained by heating the alloys to a temperature in excess of 700° C. and then quenching in water. It was found that in this way the tensile strength and 20 hardness were materially decreased while the ductility was increased, so that the quenched alloy could be cold rolled or drawn into wire or sheet form. An increase in tensile strength and hardness was obtained by heating this quenched 25 alloy for a period of time varying from 15 minutes to an hour at a temperature of from 400° to 500° C. and then allowing the alloy to cool slowly.

A considerable increase in tensile strength and 30 hardness will result if after treating at 450° C. the alloy be quenched from this temperature, but the results obtained by slow cooling from that temperature were generally superior.

The increase in hardness on the Rockwell B 35 scale is illustrated for two representative alloys in Fig. 5, the alloys having been previously treated at 860° and quenched and subsequently treated at the temperature indicated on the diagram for a period of approximately 30 minutes and 40 quenched. Curve 6 shows the results of heat treatment of an alloy of 40% Pd, 45% Ag, 15% Cu. Curve 7 represents an alloy of 40% Pd, 46% Ag, 10% Cu and 4% Ni. It is to be noted that for the alloys shown, a reheating temperature of 45 450° C. was found to produce the best results.

As an alternative heat treatment by which 50 good results are obtained, the alloy may be annealed at a temperature in excess of 700° C. and cooled from this temperature at a rate substantially slower than air cooling. The desired rate may be conveniently obtained by permitting the alloy to cool in siloel.

It has been found that an alloy having a composition of 35-55% Pd, 55-5% Ag and the remainder Cu can be given a tensile strength in 55 excess of 100,000 pounds per square inch by suitable heat treatment. As a specific instance, the influence of heat treatment on the tensile strength of an alloy containing substantially 40% palladium, 40% silver and 20% copper may be 60 noted. The ultimate strength of this alloy after quenching from 860° C. was 97,400 lbs. per square inch. After aging for 30 minutes at 450° C. and quenching, the tensile strength increased to 65 149,000 lbs. per square inch and after aging for 30 minutes at 450° C. and slow cooling, the tensile strength was increased to 171,000 lbs. per square inch.

For dental purposes it is very desirable to 70 utilize an alloy which may be hardened to a certain degree and which will be largely resistant to tarnish and corrosion. A suitable range of alloys for this purpose is represented by the area within curve FGHI of Fig. 4. It is to be noted 75 that this range is located in that area at which

substantial hardness may be obtained, as shown in Fig. 3, and in which a high degree of tarnish and corrosion resistance is obtained, as shown in Fig. 2.

In addition to the above mentioned features, 80 it has been found that the alloys described are all substantially white with practically a total absence of other colors. This white color renders these alloys especially suitable for dental purposes. Furthermore, when properly heat treated, they are of comparatively high electrical 85 conductivity, which in connection with their non-corrosive properties, renders them most suitable for electrical contacts. The density of the alloys is relatively low and therefore their costs per unit 90 volume is lower than that of many of the gold alloys which they replace.

Alloys in which palladium is present in amounts of less than 25%, possess a high heat and electrical conductivity and have a melting point 95 much higher than copper-silver alloys containing no palladium. These alloys may be useful in cases where color and tarnish resistance are of less importance.

Alloys containing 30-90% Pd with copper the 100 principal remainder may be useful for electrical contacts. Two alloys which have been found particularly suitable for this purpose comprise Pd 80%, Cu 20% and Pd 58% and Cu 42%.

In addition to the three elements, palladium, 105 silver and copper, various other elements may be present in small amounts depending upon the particular requirements of the alloy. For example, the soundness and denseness of the castings may be improved as for instance by the 110 presence of a deoxidizer such as zinc, silicon, boron, magnesium or calcium or compounds thereof. The deoxidizer should be a metal or metalloid such that the heat of formation of its oxide is substantially in excess of the heat of 115 formation of copper oxide, in order to insure the complete deoxidization of the alloy. Calcium boride in an amount of approximately .2 percent has been found suitable for this purpose.

Small amounts of other metals may be added 120 to the above alloys without departing from the spirit of the invention. Small amounts of noble metals such as gold, platinum and rhodium may be present and base metals such as nickel or cobalt may be present up to about 4%. 125

It is obvious that the compositions of the above alloys and the temperatures employed in heat treatment may vary over a wide range. Certain 130 definite figures have been given by way of example only. Furthermore, the uses of the alloy are not limited to the few instances given. They may be employed in various arts wherein their particular characteristics are of advantage.

In the initial heat treating operation the alloy may be cooled as by air cooling from a high temperature, for example 860° C. and subsequently age hardened as above described. The preferred rate of cooling in this case should be sufficient to prevent the formation of substantial amounts of a compound composed of palladium and copper 140 in the approximate ratio of their atomic weights. It has also been found that slow cooling of alloys within the hardenable range serves to increase their electrical conductivity. Alloys of 40% palladium and 5% to 20% copper, with the remainder silver, are particularly suitable for this 145 purpose and by slow cooling from a temperature in excess of 700° C. show a marked increase in electrical conductivity.

Although one process for making the improved 150

product has been set forth and described and is pointed out in the claims, it is obvious that various changes may be made in the process or in the separate steps thereof without modifying or changing the essential features and characteristics of the product produced and that such product remains substantially the same although slight modifications may be made in its appearance, texture and in its physical and chemical characteristics.

10 What is claimed is:

1. An alloy of palladium, copper and silver composed of palladium from about 25% to about 98%, copper from about 1% to about 50%, and silver not less than 1% and constituting substantially the balance, said alloy being substantially free from iron and analogous metals impairing the ductility of the alloy.
2. An alloy of palladium, copper and silver, composed of not less than 16% and not more than 48% copper, more than 33% and less than 68% of palladium, and silver to an extent of not less than 1% and constituting substantially the balance, said alloy being substantially free from iron and analogous metals impairing ductility of the alloy.
3. An alloy of palladium, copper and silver, composed of not less than 16% and not more than 50% copper, palladium ranging from about

30

35

40

45

50

55

60

65

70

35% to about 59%, and silver to the extent of not less than 4% and constituting substantially the balance, said alloy having a hardness in excess of 90 Rockwell B, and being substantially free from iron and analogous metals impairing ductility of the alloy.

4. An alloy containing 40% to 50% palladium, 14% to 30% copper and the remainder silver, said alloy being substantially free from iron and analogous metals impairing ductility of the alloy.

5. An alloy of the character set forth in claim 1, in which the deoxidizer is selected from a group consisting of manganese, zinc, silicon, boron, magnesium, calcium or compounds thereof.

6. An alloy of the character set forth in claim 1 which is adapted to be hardened by heat treatment and which contains about 25% to about 63% palladium, copper in excess of about 3.5% and less than 48% and silver not less than 1% and constituting the remainder of the alloy.

7. A non-tarnishing alloy of the character set forth in claim 1 which contains about 35% of palladium, not less than about 1% and not more than about 35% of copper, and silver constituting substantially the remainder of the alloy but being not less than 1% of the total.

EDMUND M. WISE.

80

85

90

95

100

105

110

115

120

125

130

135

140

145

150